

## 1

3,594,114

**PRETREATMENT OF DYEABLE POLYOLEFINS**  
 Albert J. Shmidl and Leroy C. Jennings, Baytown, Tex.,  
 assignors to Esso Research and Engineering Company  
 No Drawing. Filed Sept. 30, 1966, Ser. No. 583,475  
 Int. Cl. D06p 5/00

U.S. Cl. 8--168

13 Claims

**ABSTRACT OF THE DISCLOSURE**

This invention provides a method for treating a dyeable polyolefin fiber before a dyeing step, which comprises contacting the dyeable polyolefin fiber with a specific liquid treating fluid. The fluid consists essentially of 100 parts by weight made up as follows: from 98 to 80 parts by weight of acetic acid having a concentration from 40 weight percent aqueous to glacial, and from 2 to 20 parts by weight of an acid chosen from the group consisting of substantially water insoluble C<sub>6</sub> to C<sub>12</sub> alkanoic acids. The treating conditions include a pressure sufficient to maintain the treating fluid in the liquid phase, a temperature from about 75° F. to about 175° F., and a treating time from about 1 minute to about 5 minutes. Suitably, the treating step is followed by conventional acid dyeing.

The present invention is directed to an improvement in the art of dyeing polyolefins. More particularly, the present invention is directed to a pretreating step whereby polyolefins which contain basic nitrogen dyesites are given enhanced characteristics for dyeing with acid-type dyes.

Polyolefin fibers (such as polypropylene) which contain basic nitrogen dyesites (such as are provided by polyvinylpyridine) are quite easily dyed with dispersed-type dyes. The fibers are not readily dyed however, with acid-type dyes, which, because of their good stability against fading in sunlight, are preferred for many uses.

Dyeable polyolefins have been pretreated with Lewis acids to enhance their dyeability with acid-type dyes. Glacial acetic acid has been employed for this purpose. As will be seen hereinafter, the present invention is an improvement over that process (described in the U.S. Rubber South African application 62/5464). The present process makes more practicable the use of dyeable polyolefins as synthetic fibers.

One of the objectives of the polyolefin industry has been to produce a fiber which is susceptible to treatment in the same manner as competing fibers when used in woven goods. Polyolefin fibers have a number of advantages over the natural fibers, including a resistance to moisture and mildew which cannot be obtained in wool or natural fibers. However, polyolefins suffer from one major drawback; that is, the polyolefin (such as polypropylene) is a hydrocarbon and does not contain a dyesite which is susceptible of reaction with a dye. Thus, the prior art has utilized a practice of compounding the fibers with colored pigment fillers, or dyeing the polyolefin by dissolving a coloring agent into the amorphous regions of the polymer. Neither expedient has been entirely successful.

In the commercial practice of using dyeable fibers such as wool, natural fibers, etc., the raw fibers are usually spun and woven before being submitted to a dyebath, so that a woven fabric is first obtained prior to dyeing. If the results of the dyebath are unsatisfactory for any reason, the fabric can be bleached and redyed by the manufacturer. The previously used blends of polypropylene with pigments are not susceptible to bleaching, and the polypropylene containing dissolved dyes is not resistant to leaching during laundering.

If polyolefins are to compete in the market with natural and synthetic fibers, they must be prepared in a

## 2

manner which allows them to be dyed and bleached in a manner analogous to the treatment of the natural fibers. The preparation of a polyolefin which contains basic nitrogen dyesites has been suggested. First, dyesites can be incorporated by copolymerization of a vinyl compound (having a basic nitrogen substituent) with the olefin monomer in order to incorporate the dyesite into the structure of each polymer chain. A second manner in which the dyesite can be incorporated is by physically blending with the homopolymer a material which does contain dyesites. For example, small amounts of a polyvinylpyridine can be blended into the homopolymer. A third manner of incorporating dyesites within the polyolefin fiber is by a graft polymerization, such as the polymerization of styrene and a maleic anhydride upon the chain of a polypropylene homopolymer. It has also been suggested that polyvinylpyridine can be grafted upon the chain of a polypropylene homopolymer.

The net result of all of these attempts to introduce reactive dyesites into the polyolefin itself is to distribute basic nitrogen dyesites throughout the polymer. When the polymer is drawn into a fiber, this results in a distribution of at least a part of the dyesites at or near the surface of the fiber. From the standpoint of economics, it is usually desirable to keep the amount of the added dyesites at a practical minimum. Where the basic nitrogen dyesite is employed, it is usually employed in amounts within the range from 0.05 to 0.5 weight percent of nitrogen, based on the weight of the entire polymer. Nitrogen levels above 0.5 weight percent can be used, but are not as economically attractive as the lower levels, and in some cases can result in an impairment of the physical property of the resulting fibers.

At the low concentrations of basic nitrogen dyesites which are employed, there is a real problem involved in attempting to reach the dyesites with the dye in the aqueous dyebath which is employed. Only a small portion of the dyesites would appear at the surface of the fiber, and those which are internal of the fiber cannot be contacted unless the dye itself penetrates into the fiber. This presents problems of uneven dyeing, resulting in barre or spotted appearance of the resulting fabric.

It has been suggested by U.S. Rubber in its South African application 62/5464 that a polyolefin blended with polyvinylpyridine can be pretreated by reaction with a Lewis acid before introduction into the dyebath. This "activates" the polymer for reaction with acid-type dyes. The U.S. Rubber application suggests the use of a number of widely different Lewis acids, among which are organo-carboxylic acids, such as formic, acetic, propionic and other alkanoic acids in the C<sub>1</sub> to C<sub>18</sub> range, as well as stearic, undecylenic, oleic, benzoic, etc., acids. These acids are suggested for use as such or in a water solution containing at least 20% concentration of the acids. The fiber or fabric is first treated with the acid solution, and is thereafter introduced into the dyebath.

Although the pretreatment process suggested by U.S. Rubber results in an improved dyeing of the fabric, the use of concentrated acids (such as glacial acetic acid) leaches additives (e.g., antioxidants) from the fibers, while the use of dilute acids has been, in general, unsatisfactory. The present invention allows the use of dilute acetic acid and lower temperatures in accomplishing a commercially acceptable dyeing process.

Before proceeding to a specific discussion of the manner in which the present invention is carried out, it should be understood that the following terms wherever used in the present application have the meanings set forth below:

The term "fiber" shall mean a filament, drawn or un-drawn, in the form of discrete filaments, yarn, or woyen fabric material.

The term "polyolefin" shall mean a solid hydrocarbon polymer, stabilized or unstabilized, containing poly- $\alpha$ -olefins, such as polyethylene, polypropylene, polyisobutene, poly-1-butene, etc.; polydolefins, such as poly-1,4-buta-  
diene, etc.; and other polymers, such as polystyrene, etc., either as the homopolymer, as a blend of homopolymers (for example, polyethylene and polypropylene or polypropylene and polyisobutene), or as an olefinic copolymer, such as ethylene-propylene random copolymer, ethylene-propylene block copolymer, etc., including ethylene-propylene rubber. When reacted or blended with a material containing basic nitrogen dyesites, the material is referred to as a "dyeable polyolefin."

The term "dyesites" refers to reactive portions incorporated into the polymer which aid in retaining the dye to be used, and is preferably an amino nitrogen, and (as applied to the present invention) in all cases will be a basic nitrogen.

The term "dyesite additive" refers to a material containing dyesites which is blended with a polyolefin in order to provide dyesites.

The term "acid-type dye" is to be considered to include both the acid dyes and the premetallized dyes which fall under the usual definition of an acid-type dye: "a dye which will dye wool from an acid bath."

#### TYPES OF DYEABLE POLYOLEFINS

The polyolefins to which the present invention is particularly directed are those which basically contain only hydrogen and carbon, such as polyethylene, polypropylene, ethylene-propylene copolymers, polyisobutene, polyisoprene, etc. As such, they contain no dyesites and cannot be successfully dyed. Dyesites may be chemically incorporated into the polyolefins by copolymerizing the olefin monomers with small amounts of dyesite-containing monomers; that is (using polypropylene as an example), both propylene and a dyesite-containing monomer (such as an alkenyl amine) may be introduced into the polymerization zone to obtain a polymer which has dyesites as a part of the polymer structure. This type of dyeable polypropylene is exemplified by a propylene-N,N-diisopropyl-7-octenylamine copolymer containing 0.06 weight percent nitrogen.

Alternatively, the dyesite-containing monomer may be grafted onto the polypropylene after polymerization, as exemplified by polypropylene with polyvinylpyridine engrafted thereupon.

Other variants include physical blends of polymers (such as polypropylene) with materials containing dyesites, such as copolymers containing reactive dyesites in the chain (similar to the octenyl amine-propylene polymer described above) or with other organic or inorganic materials which provide such dyesites (such as polyvinylpyridine). The relative proportions in these blends will depend on a balancing of a number of factors, including the effect of the blend stock on polymer properties, intensity of color required, efficiency of dyesite additive, etc. The particular additive to be used will depend on the type of dye to be employed, the use to which the dyed material will be put, etc.

All of these modified fibers are referred to herein as "dyeable polyolefins." The process of the present invention is equally applicable to films and fibers, drawn and undrawn, woven and unwoven, which are made from resins of the dyeable polyolefins.

#### ACID DYES

The present invention contemplates the use of acid-type dyes. As used in this application, the acid-type dye will include the premetallized dyes. As examples of the dyes that are useful in this process, and as incorporated in the dyeing composition, are the following dyes as set forth in Table I. The color index, where available, is shown in parentheses.

4  
TABLE I  
Dye

|    |                                                  |
|----|--------------------------------------------------|
|    | Acid dyes:                                       |
| 5  | Erio Anthracene Rubine 3 GP—(Acid Red 57).       |
|    | Erio Fast Violet LN—(61700).                     |
|    | Erio Anthracene Brilliant Blue 2 GC—(62055).     |
| 10 | Erio Fast Brown 5 RL                             |
|    | Duronylan Scarlet LVGGL                          |
|    | Duronylan Brilliant Blue LVGF                    |
|    | Duronylan Black LVTRR                            |
|    | Irganol Scarlet RLS                              |
|    | Alizarine Light Green GSN—(Acid brown 25;61570). |
| 15 | Wool Fast Blue HFL—(AB-25).                      |
|    | Premetallized dyes:                              |
|    | Levalan Navy Blue IRL                            |
|    | Levalan Olive I-GL                               |
|    | Irganol Brilliant Yellow 3 GLS—(AY 127).         |
|    | Irgalan Violet 5 RL                              |
|    | Chromolan Orange R                               |
|    | Chromolan Black NWA—(Acid Black 52;15711).       |
|    | Vialon Fast Yellow G—(HY 118).                   |
| 20 | Vialon Fast Red B—(AR 225).                      |
|    | Vialon Fast Violet B                             |
|    | Vialon Fast Green FFG                            |
|    | Vialon Fast FFG                                  |
|    | Vialon Fast Brown R                              |
| 25 | Vialon Fast Blue Grey B—(AB-61).                 |
|    | Vialon Fast Red G                                |
|    | Vialon Fast Violet RR                            |
|    | Vialon Fast Black R—(AB-63).                     |
|    | Avilan Fast Scarlet 2 R                          |
|    | Avilan Fast Navy Blue BW                         |
|    | Avilan Fast Black B                              |
|    | Avilan Fast Red GW                               |
|    | Avilan Fast Violet 3B                            |
|    | Avilan Fast Navy Blue R                          |
|    | Avilan Fast Olive GW                             |
| 30 | Lanamid Red GL                                   |
|    | Lanamid Blue BL                                  |
|    | Lanamid Dark Green                               |
|    | Lanamid Brown BL—(AB-19).                        |
|    | Lanamid Bordeaux BL                              |
|    | Isolan Red 2G                                    |
|    | Isolan Black BGL                                 |
|    | Irgalan Violet 5RL                               |
|    | Irgalan Blue RL                                  |
|    | Irgalan Brilliant Green 3GL                      |
| 35 | Irgalan Dark Brown SR                            |
|    | Lanasyn Dark Violet RL                           |
|    | Lanasyn Brown RL                                 |
|    | Lanasyn Black BGL                                |
|    | Lanasyn Yellow 2GW—(AY 129).                     |
| 40 | Lanasyn Brilliant Blue GL                        |
|    | Lanasyn Olive 2GL                                |
|    | Cibalan Blue BRL                                 |
|    | Atalan Red 2GA                                   |
|    | Atalan Blue GA                                   |
|    | Vitrolan Bordeaux RM                             |
| 45 | Ortalan Violet B                                 |
|    | Ortalan Black G Special                          |
|    | Capracyl Blue G                                  |
|    | Neolan Blue 2G—(AB 158;14880).                   |
|    | Neolan Green 8G—(Acid Green 24).                 |
| 50 | Neolan Brown GR                                  |
|    | Sandolan Dark Brown GL                           |
| 55 |                                                  |
| 60 |                                                  |
| 65 |                                                  |
| 70 |                                                  |
| 75 |                                                  |

As can be seen by reference to the above table, the present invention involves the use of acid and premetallized dyes to obtain a more effective dyeing of dyeable polyolefins.

In using the dye, it is employed generally in accordance with instructions provided by the manufacturer. Generally, the dyes will be used in suspension or in solu-

tion in a hot aqueous dyebath. The premetallized dyes are employed in an aqueous dispersion, being in a concentration of 1.0 to 5.0 weight percent O.W.F. (that is, based on the weight of the fiber to be dyed in the dyebath). A dispersing agent can be employed as herein-after described, preferably being added to the dyebath in an admixture with the treating acid. The dyebath is kept at a temperature of 100° to 212° F., and the fabric is contacted with the dyebath for a period of time determined by the type of fiber employed in the fabric, type of dye employed, the depth of color desired, dye concentration, etc. The pH in the dyebath will vary, depending on the particular dye being employed and the desire of the dyer. The pH may be adjusted by adding a C<sub>1</sub> to C<sub>3</sub> alkanoic acid, or a dilute mineral acid such as sulfuric acid, either at the beginning of the dyeing process in sufficient quantities to maintain the pH at the desired level, or by gradual addition during the conduct of the dyeing process. For low pH dyeing, the use of formic acid is preferred, since it is possible to obtain a pH of 3.0 while using 3% formic acid (based on the weight of the fiber) as compared to about a 3.5 pH when employing similar amounts of acetic acid.

#### PRETREATING FLUID

The present invention contemplates the use of a novel pretreating fluid. This fluid is made up of two constituents: (1) a water-soluble acid (acetic acid) and (2) a substantially water-insoluble acid such as octanoic acid. This treating fluid allows the treatment of fibers to be accomplished at lower temperatures or with dilute (rather than glacial) acetic acid, thus minimizing the extraction from the fiber of constituents added to the polyolefin for inhibition of oxidation, etc.

The treating fluid can be made up of acetic acid having a concentration from 40% aqueous to glacial. This acetic acid can be mixed with from 2 to 20 weight percent (based on the resulting mixture) of a C<sub>6</sub> to C<sub>12</sub> substantially water-insoluble alkanoic acid (or substituted derivative thereof). Above 15 weight percent, there is no appreciable improvement. Suitable alkanoic acids are hexanoic, heptanoic, octanoic, nonanoic, decanoic, undecanoic, and dodecanoic acids, and the isomers thereof. Using octanoic acid as an example, the treating fluid might have the following formulations:

#### I

|                     | Parts by weight |
|---------------------|-----------------|
| Glacial acetic acid | 90              |
| Octanoic acid       | 10              |

#### II

|                                    | Parts by weight |
|------------------------------------|-----------------|
| 40 wt. percent aqueous acetic acid | 90              |
| Octanoic acid                      | 10              |

#### THE METHOD OF PRETREATING

A dyeable polyolefin fiber, e.g. in a woven fabric, is contacted with the treating fluid by immersion or by spraying. The fiber is maintained in contact with the treating fluid for a period of from about 1 minute to about 5 minutes, at a temperature from about 75° F. to about 175° F., and a pressure from 0 p.s.i.g. to 25 p.s.i.g. (preferably, by immersion for about 2 minutes at 140° F., atmospheric pressure). Pressure is not critical, so long as the treating fluid is maintained in the liquid phase. The preferred treating fluid, for use under preferred conditions, will be made up of about 90 parts by weight of 40% aqueous acetic acid and 10 parts by weight of octanoic acid.

After pretreatment, the fiber is removed from contact with the treating fluid and is dyed in the regular manner with an acid-type dye. Excess treating fluid may be removed from the fibers by sponging or by allowing the fibers to drip-dry, if desired. The fibers may, however, be placed in the dyebath without a deliberate attempt to remove the excess fluid if the resulting loss of fluid is not uneconomical.

#### DYEING

The dyeing step is carried out as usual. Normally, the specific conditions are recommended by the manufacturer of the dye which is employed. In general, dyeing conditions will include a dyebath made up as follows:

Water: 20-50 (preferably 30) parts/part of fiber  
Dye: 1-5 wt. percent (preferably 3 wt. percent) O.W.F.  
Dispersant: 0.5-1 wt. percent (preferably 0.5 wt. percent)

O.W.F.

pH: 2.7 to 5.0 (preferably 3.7)

The temperature is usually from 200° to 212° F. (preferably 208° F.) and the pressure is usually atmospheric. The dyeing time (measured from the time the dyebath reaches the dyeing temperature) may be from 20 to 90 minutes, preferably about 30 minutes.

The dyebath is first made up, then the fiber is introduced. The dyebath is then heated, under mild agitation or fluid circulation, to the dyeing temperature. After the dye has been absorbed by the fiber, the fiber is removed from the dyebath, scoured, and dried.

#### EXAMPLES

In the following examples, 99 parts of polypropylene (melt index 12) were blended with about 1 part of a polyvinylpyridine copolymer derived from equimolar parts of 2-methyl-5-vinylpyridine and 2-vinylpyridine, having a molecular weight of about 40,000. The blend contained about 0.15 weight percent nitrogen based on the weight of the entire blend.

##### Example 1

The fiber was treated at atmospheric pressure by immersion for 2 minutes in glacial acetic acid at 140° F. This fiber dyed to a fair blue with 2% O.W.F. Erio Anthracene Brilliant Blue 2GC, an acid dye.

##### Example 2

The fiber was treated at 140° F. and atmospheric pressure by immersion for 2 minutes in an admixture of 90 parts of glacial acetic acid and 10 parts of octanoic acid. This fiber dyed to about three times the color intensity of that shown in Example 1 when dyed under the same dyeing conditions with the Erio Anthracene Brilliant Blue 2GC.

##### Example 3

The fiber was treated with the admixture of acids as in Example 2 for 2 minutes at room temperature (about 75° F.). It showed more dye receptivity for the same blue acid dye than the fiber of Example 1.

##### Example 4

The fiber was treated with an admixture of 86 parts of 50% aqueous acetic acid and 14 parts of octanoic acid, under the same conditions as Example 1, and was then dyed with a premetallized dye, Vialon Fast Violet RR. The sample showed a deeper color uptake than a companion sample treated with glacial acetic acid under the conditions of Example 1.

The various test samples are shown in color in the attached affidavit under Rule 132, which is hereby incorporated by reference into this disclosure.

Having disclosed our invention, and the preferred mode and embodiment thereof, we claim:

1. A method of treating a dyeable fiber consisting essentially of a blend of a polyvinylpyridine in a poly- $\alpha$ -olefin in an amount sufficient to provide between 0.05 to 0.5 weight percent nitrogen, based on the weight of the entire blend, which comprises

in a treating zone, contacting said dyeable fiber with a liquid treating fluid prior to dyeing of said fiber, said treating fluid consisting essentially of 100 parts by weight as follows:

from 98 to 80 parts by weight of acetic acid having a concentration from 40 weight percent aqueous to glacial, and

- from 2 to 20 parts by weight of an acid chosen from the group consisting of substantially water-insoluble  $C_6$  to  $C_{12}$  alkanoic acids under treating conditions including a pressure sufficient to maintain the treating fluid in the liquid phase, a temperature from about 75° F. to about 175° F., and a treating time from about 1 minute to about 5 minutes.
2. A method in accordance with claim 1 wherein the alkanoic acid is octanoic acid.
3. A method in accordance with claim 1 wherein the alkanoic acid is isodecanoic acid.
4. A method in accordance with claim 2 wherein the constituents are as follows: 90 parts by weight of glacial acetic acid and 10 parts by weight of octanoic acid.
5. A method in accordance with claim 2 wherein the constituents are as follows: 90 parts by weight of 40 weight percent aqueous acetic acid and 10 parts by weight of octanoic acid.
6. A method in accordance with claim 2 wherein the constituents are as follows: 86 parts by weight of 50 weight percent aqueous acetic acid and 14 parts by weight of octanoic acid.
7. A method of dyeing a dyeable fiber consisting essentially of a blend of a polyvinylpyridine in a poly- $\alpha$ -olefin in an amount sufficient to provide between 0.05 and 0.5 weight percent nitrogen, based on the weight of the entire blend, which comprises in a treating zone, contacting said dyeable fiber with a liquid treating fluid, said treating fluid consisting essentially of 100 parts by weight, as follows: from 98 to 80 parts by weight of acetic acid having a concentration from 40 weight percent aqueous to glacial, and from 2 to 20 parts by weight of a substantially water-insoluble  $C_6$  to  $C_{12}$  alkanoic acid under treating conditions including a pressure sufficient to maintain the treating fluid in the liquid phase, a temperature from about 75° F. to about 175° F., and a treating time from about 1 minute to about 5 minutes, separating the resulting treated fiber from said treating fluid, and thereafter in a dyeing zone, under dyeing conditions, contacting said treated fiber with an acid-type dye in an aqueous dyebath, said aqueous dyebath containing from 1 to 5 weight percent O.W.F. of acid dye, from 0.5 to 1 weight percent O.W.F. of a dispersant, and said dyeing conditions including a pressure sufficient to maintain the dyebath in the liquid phase, a temperature from 200° to 212° F., a pH from 2.7 to 5.0, and a dyeing time from 20 to 90 minutes.
8. A method in accordance with claim 7 wherein the alkanoic acid is octanoic acid.
9. A method in accordance with claim 7 wherein the alkanoic acid is isodecanoic acid.
10. A method of treating a dyeable fiber, said fiber consisting of from 0.5 to 3 weight percent polyvinylpyridine blended into polypropylene, which comprises in a treating zone, contacting said dyeable fiber with a liquid treating fluid prior to dyeing of said fiber,

- said treating fluid consisting essentially of 100 parts by weight, as follows: from 90 to 86 parts by weight of acetic acid having a concentration from 40 weight percent aqueous to glacial, and from 10 to 14 parts by weight of an acid chosen from the group consisting of octanoic acid and isodecanoic acid under treating conditions including a pressure sufficient to maintain the treating fluid in the liquid phase, a temperature from about 75° F. to about 175° F., and a treating time from about 1 minute to about 5 minutes.
11. A method in accordance with claim 10 wherein the acid is octanoic acid.
12. A method of dyeing a dyeable fiber, said fiber consisting of from 0.5 to 3 weight percent polyvinylpyridine blended into polypropylene, which comprises in a treating zone, contacting said dyeable fiber with a liquid treating fluid, said treating fluid consisting essentially of 100 parts by weight, as follows: from 90 to 86 parts by weight of acetic acid having a concentration from 40 weight percent aqueous to glacial, and from 10 to 14 parts by weight of an acid chosen from the group consisting of octanoic acid and isodecanoic acid under treating conditions including a pressure sufficient to maintain the treating fluid in the liquid phase, a temperature from about 75° F. to about 175° F., and a treating time from about 1 minute to about 5 minutes,
13. A method in accordance with claim 12 wherein the acid is octanoic acid.

#### References Cited

##### UNITED STATES PATENTS

- 60 3,231,530 1/1966 Prahl ----- 8—55  
3,361,843 1/1968 Miller et al. ----- 260—895

##### FOREIGN PATENTS

- 65 1,388,253 12/1964 France ----- 8—55  
752,759 2/1967 Canada.

##### OTHER REFERENCES

- K. S. Markley: "Fatty Acids," Interscience Pub., N.Y., 1960, pp. 609, 633, 639, 647.

- 70 NORMAN G. TORCHIN, Primary Examiner  
C. L. BOWERS, Jr., Assistant Examiner